

Feb. 13, 1940.

J. H. MCGILL

2,189,811

HEEL CONSTRUCTION

Filed Aug. 9, 1937



INVENTOR  
John H. McGill  
By his attorney  
Victor Colb.

## UNITED STATES PATENT OFFICE

2,189,811

## HEEL CONSTRUCTION

John H. McGill, Winchester, Mass., assignor to  
 B. B. Chemical Co., Boston, Mass., a corpora-  
 tion of Massachusetts

Application August 9, 1937, Serial No. 158,016

1 Claim. (Cl. 36—42)

This invention relates to shoe heels and more particularly to heel constructions embodying detachable leather top lifts.

An object of this invention is to provide a heel construction embodying a detachable leather top lift which may be readily removed after it has become worn. A further object is to provide a heel construction embodying a detachable leather top lift arranged to exhibit a uniformly good appearance throughout the life of the lift.

In accordance with the above and other objects we have provided by the present invention a heel construction embodying a detachable leather top lift wherein at least the flesh side of the lift contiguous to the lower or lift-receiving surface of a wood heel is hardened or stiffened by incorporating in the leather molten thermoplastic material selected from the group of substances consisting of waxes and resins. The impregnation by the molten wax or resin or mixture thereof preferably takes place on the flesh side of a leather lift and may extend to any desired extent therefrom. The impregnation advantageously may take place from the edges as well as the flesh side of the lift. In certain cases impregnation of the lift may take place from all the surfaces thereof including the grain side. Leather top lifts treated in the manner described are hardened and stiffened on the flesh side of the lift so as to provide an excellent bearing surface for a tool inserted between the lift and the heel in removing a worn lift for replacement. Moreover, portions of the lift impregnated with the molten wax or resin exhibit substantial resistance to fraying when subjected to wear. Lifts so treated readily may be finished with the usual leather finishes and exhibit an excellent appearance. Furthermore, the portions of a lift treated with the molten wax or resin exhibit a considerably greater resistance to the detanning and disintegrating action of water than lifts not so treated. Generally speaking, in the heel construction contemplated by this invention, except for the hardening and stiffening action of the molten wax or resin, leather top lifts exhibit the general characteristics of leather.

In the drawing,

Fig. 1 is a perspective view of a treated leather top lift secured to a post;

Fig. 2 is an elevation, partly in vertical section, illustrating the improved heel construction of this invention;

Fig. 3 is a fragmentary vertical section of a detachable top lift and adjacent portions of a wood heel illustrating the impregnation of the

lift with molten wax or resin from the flesh side only of the lift and to a relatively slight extent; and

Fig. 4 is a fragmentary vertical section similar to Fig. 3 and illustrating a relatively deep impregnation of the top lift from the flesh side with molten wax or resin.

In the embodiment of the invention illustrated in Figs. 1 and 2 there is shown a shoe 2 to which is secured a wood heel 4. The wood heel 4 is provided with a receiving socket 6 lined with a metallic sleeve 8. Arranged to be held by friction or other means within the receiving socket 6 and sleeve 8 is the post 10 provided with prongs 11 which extend into the substance of the leather top lift 12 and are upset therein to provide a mechanical attachment of the post 10 to said lift 12, the upper or flesh side 14 and edges 15 of which lift have been impregnated with molten wax or resin to render the same relatively stiff and hard but otherwise retaining essentially the characteristics of leather. The wax or resin 17 extends downwardly toward the grain or lower side 16 of the lift 12.

In the modification shown in Fig. 3 the wax or resin 17 is shown as impregnating the lift 18 only from the upper or flesh side 20 thereof and merely to a slight extent.

In the modification shown in Fig. 4 the wax or resin 17 is shown as impregnating the lift 22 from the upper or flesh side 24 thereof to an extent closely approaching the lower or grain side 26 thereof whereby the edges 28 are also impregnated to a substantial extent.

In all of the above cases the prongs 11 of the post 10 readily may be incorporated in the substance of the impregnated top lifts and upset therein to provide a secure anchorage. This is due to the fact that except for the hardening and stiffening effect of the impregnated molten wax or resin the lifts retain the essential properties of leather.

In view of the fact that the upper or flesh sides of the top lifts remain firm and hard throughout the life of the lifts, there is provided in all of the modifications of top lifts illustrated a firm bearing surface for the insertion of a tool between the top lift and the lower or top-lift-receiving surface 30 for ready removal of the lift when replacement thereof is desired.

The edges of the top lift illustrated, slightly impregnated with wax or resin as in Fig. 3, or impregnated with wax or resin to a greater extent as in Figs. 2 and 4, take edge inks and leather finishes as satisfactorily as or even better than

top lifts not so treated whereby a highly desirable top lift appearance is provided for the shoe which remains throughout the life of the lift.

Furthermore, where the edges of the top lift are impregnated to a substantial extent, as illustrated in Figs. 2 and 4, such impregnated portions exhibit little if any fraying when the lift has worn down to such portions.

The impregnation of the top lifts by molten wax or resin may be accomplished in the manner disclosed in my copending application, Serial No. 158,017, filed August 9, 1937, in which said application the method of impregnation and articles resulting therefrom are claimed.

As disclosed in my said copending application, the impregnation of the flesh side and edges of the lift 12 illustrated in Figs. 1 and 2 may be accomplished by supporting the heel lift, flesh side downward, at a predetermined level in a bath 20 of molten carnauba wax, cumar resin, or a combination of 60% montan wax and 40% M rosin, maintained at a temperature of about 110° to 130° C., and permitting said heel lift to remain in said bath for 3 to 5 minutes.

The impregnation of the lift 18 on the flesh side 20 only and to a slight extent (Fig. 3) may be accomplished by supporting a piece of leather stock in a molten wax or resin bath at the desired level and later dieing or cutting out the lift 18 from the impregnated leather stock.

The relatively deep impregnation of the lift 22 illustrated in Fig. 4 may be accomplished by supporting a leather lift in a molten wax or resin bath for a sufficient time to accomplish the impregnation to the desired extent or by impregnating a larger piece of leather stock and dieing or cutting out the lift therefrom.

In the lifts illustrated in the drawing it will be noted that the grain side of the lift is left in

its original condition whereby the natural leather finish or any other desired finish may be imparted to the grain side of the lift. In certain cases, however, it may be desired to impregnate the lift from all the surfaces thereof including the grain side which may be accomplished by completely immersing the lift or a piece of leather stock in a molten wax or resin bath until the desired impregnation has been accomplished.

Furthermore, as disclosed in my said copending application, Serial No. 158,017, there may be incorporated in the molten wax, resin, or mixture thereof, a small percentage of a compatible dye for the purpose of imparting a permanent color to the impregnated portion of the leather. 15 By way of example, 3% of oil black dye may be associated with 97% montan wax.

Having described my invention, what I claim as new and desire to secure by Letters Patent of the 20 United States is:

A shoe heel construction comprising a wood heel provided with a receiving socket, a post, a leather top lift secured to said post, said post being arranged to fit tightly into said receiving socket and to hold the lift with the flesh side 25 thereof adjacent to the lower or top-lift-receiving surface of said heel, the upper or flesh side and the edges of said heel lift from the flesh side to a point short of the grain side being impregnated with material from the group consisting of waxes 30 and resins, and the lower or grain side of said heel lift being free from said waxes and resins, whereby the grain side of the lift is preserved in its original condition, and the associated lift and post readily may be removed by insertion of 35 a tool between the lift and the contiguous lift-receiving surface of the heel.

JOHN H. MCGILL.